

## 1

2,852,380

PHOTOGRAPHIC EMULSIONS AND SOLUTIONS  
CONTAINING SILVER SALTS OF THIOLY-  
COLIC DERIVATIVES

Henry C. Yutzy and Albert W. Wise, Rochester, N. Y.,  
assignors to Eastman Kodak Company, Rochester,  
N. Y., a corporation of New Jersey

No Drawing. Application June 21, 1955  
Serial No. 517,092

6 Claims. (Cl. 96—96)

This invention relates to photographic products in which silver salts of thioglycolylamidobenzothiazole or of acetylthioglycolylamidobenzothiazole are incorporated to prevent "plumming" or "bronzing" of the photographic image during ferrotyping.

Silver halide emulsions are frequently subject to image degradation during processing and during ferrotyping or hot glazing. This deterioration of the photographic image frequently manifests itself as plumping or bronzing of the image during ferrotyping.

U. S. 2,657,135 of Lowe and Hamshire describes a procedure for preventing the plumping of photographic prints during ferrotyping. That method involves the carrying out of one of the steps of processing exposed silver halide emulsion in the presence of a thioglycolic amide derivative. The method described therein is effective for that purpose but in the case of some types of silver halide emulsions desensitizing of the emulsion may occur when compounds of the type mentioned therein are contacted with the silver halide for extended periods.

One object of our invention is to provide a method of preventing plumping of photographic silver images without decreasing the sensitivity of the silver halide emulsion from which they are derived. Another object of our invention is to employ certain simple salts to give the antiplumping effect. A further object of our invention is to provide antiplumping agents which may be directly incorporated in the photographic emulsion or in layers in contact therewith without any effect upon the properties of the photographic emulsion. Other objects of our invention will appear herein.

We have found that the silver salt of 2-thioglycolylamidobenzothiazole and the silver salt of 2-acetylthioglycolylamidobenzothiazole are both excellent antiplumping agents either when added to the photographic emulsion prior to applying to a support or when incorporated in a gelatin solution which is applied as an overcoating over the photographic emulsion layer. We have found that the tendency of thioglycolic acid derivatives to desensitize fast emulsions is eliminated by using the silver salts in contact with the photographic emulsion either by incorporating therein or by incorporating in layers in contact with photographic emulsion layers.

Our invention involves the reacting of silver nitrate with sodium salts of the compounds listed, or with the compounds themselves, and incorporating the so-formed silver derivatives either into the photographic emulsion or into gelatin compositions which are employed for coating purposes. We have found that by thus incorporating the so-formed silver derivatives either in the emulsion or in the layers adjacent thereto that no desensitizing effect is observed even in the case of emulsions having highly sensitive characteristics, and that, upon ferrotyping photographic prints made therefrom, the maximum den-

## 2

sity obtained is consistently better than the corresponding maximum density when these compounds are omitted or when the free compounds corresponding thereto are incorporated in the emulsion layer or in coating layers adjacent to the photographic emulsion layer. Compounds whose silver salts are useful in products in accordance with our invention are described in U. S. Patent 2,503,861 of Weissberger of April 11, 1950. The compounds in accordance with our invention are employed at the rate of 0.5—3 grams of silver salt per mol of silver halide contacted in accordance with our invention.

The following examples illustrate our invention.

## Example 1

Finely dispersed silver chloride was prepared by adding a solution of 5.44 grams of silver nitrate in 95 ml. of water and a solution of 2.24 grams of potassium chloride in 95 ml. of water simultaneously to 200 ml. of 5% gelatin solution at 40° C. with stirring. The silver salt of 2-thioglycolylamidobenzothiazole was formed by mixing a solution of the sodium salt thereof (which had been prepared by dissolving 2.6 grams of 2-acetylthioglycolylamidobenzothiazole in 14 ml. of 2.5 N. sodium hydroxide with 25 ml. of additional water) with the silver chloride preparation. The thus prepared silver salt was added to a gelatino-silver chloride emulsion containing about 2% silver bromide, in one case in the proportion of 0.7 gram of the silver salt of acetylthioglycolylamidobenzothiazole per mol of silver halide and in the second case in the proportion of 2.8 grams thereof per mol of silver halide in the emulsion. Solutions of saponin and formaldehyde were also added to each sample of emulsion and they were coated on a single weight baryta coated paper at the rate of 1 mol of silver per 1000 sq. ft. The product was exposed, developed, fixed and washed and test strips were dried at approximately 190° F. on a Kodak gloss print drier. The results obtained as compared with the same emulsion having no antiplumping agent therein were as follows:

| Concentration of anti-plumping agent—grams per mol of silver | Maximum density after drying at 190° F. |
|--------------------------------------------------------------|-----------------------------------------|
| 0.....                                                       | 1.43                                    |
| 0.7.....                                                     | 1.71                                    |
| 2.8.....                                                     | 1.78                                    |

## Example 2

A sodium salt of thioglycolylamidobenzothiazole was prepared by dissolving .005 mol of acetyl thioglycolylamidobenzothiazole in 2.5 normal NaOH. The sodium salt was added to a solution containing 5 grams of gelatin, 10 ml. of 7.5% saponin and sufficient water to make 313 ml. There was then added thereto with stirring a silver nitrate solution containing 0.74 gram silver nitrate, 5 grams gelatin, 10 ml. of 7.5% saponin and sufficient water to make 312 ml. There was thereby obtained a suspension of silver salt in aqueous gelatin. This material was coated over a gelatino-silver chloride emulsion containing 2% silver bromide at rates equivalent to 2.0, 5.5 and 15 mg. of the silver salt of thioglycolylamidobenzothiazole per sq. ft., the emulsion layer being present on the paper at the rate of 1 mol of silver per 1000 sq. ft. After drying, the photographic product thus obtained was exposed, developed, fixed and washed and test strips were dried at 195° F. on a Kodak gloss print drier. The effectiveness of the silver salt in sup-

pressing the loss in maximum density due to heat drying as compared to a control in which no antiplumming agent was used is as follows:

| Concentration of anti-plumming agent, Milligrams per Sq. Ft. or grams per mol of AgX | Maximum Density After Drying at 185° F. |
|--------------------------------------------------------------------------------------|-----------------------------------------|
| 0.....                                                                               | 1.74                                    |
| 2.0.....                                                                             | 2.00                                    |
| 5.5.....                                                                             | 2.12                                    |
| 15.....                                                                              | 2.10                                    |

AgX being silver halide.

*Example 3*

A silver salt of acetylthioglycolylamidobenzothiazole was prepared by dissolving 0.675 g. thereof in 100 ml. of methanol, mixing with 187 grams of 6.6% gelatin solution plus sufficient water to bring the total volume to 375 ml. and mixing the whole with a second solution of 44 ml. of 1% silver nitrate solution, 187 ml. of 6.6% gelatin solution mixed with sufficient water to bring the total volume to 375 ml. The solution of silver nitrate was added quickly and with stirring to the solution of acetylthioglycolylamidobenzothiazole.

The silver salt in gelatin solution thus prepared was applied over a gelatin silver chloride emulsion layer on single weight baryta coated paper base at a rate equivalent to 7.5 mg. of the silver salt of acetylthioglycolylamidobenzothiazole per sq. ft., the emulsion coating being at the rate of approximately 1 mol of silver per 1000 sq. ft. Another application of the silver salt at the rate of 3.75 mg. per sq. ft. was made by first diluting the solution of gelatin and silver salt with an equal volume of 3.3% gelatin solution. These products were exposed and were developed, fixed and washed. Test strips of this photographic material were dried at 180° F. on a print drier and the table indicates the comparison of the maximum density of the product as compared to one in which the antiplumming agent was not supplied.

| Concentration of silver salt antiplumming agent | Maximum density after hot ferrotyping |
|-------------------------------------------------|---------------------------------------|
| 0.....                                          | 1.73                                  |
| 3.75 mg. per sq. ft. or 3.75 g./mol AgX.....    | 1.96                                  |
| 7.5 mg. per sq. ft. or 7.5 g./mol AgX.....      | 2.11                                  |

AgX being silver halide.

*Example 4*

The silver salt of thioglycolylamidobenzothiazole causes no desensitization when material containing that salt is coated over an enlarging speed silver bromoiodide emulsion while the sodium salt of the thioglycolyl compound causes considerable desensitization.

Overcoating solutions containing the sodium salt and the silver salt of thioglycolylamidobenzothiazole were prepared as described in Example 2. Each salt was coated at a rate equivalent to 2.0 mg. of thioglycolylamidobenzothiazole per sq. ft. over a silver bromoiodide emulsion containing approximately 1.3 mol percent of silver iodide and having a speed suitable for exposing in a Photostat Camera. One mol of the emulsion was coated over 500 sq. ft. After exposure, development, 60

65

fixation and washing, test strips were dried at approximately 290° F. The results obtained in the 2 cases are as follows:

| 5  | Overcoat containing— | Relative Speed | Maximum density after drying at 290° F. |
|----|----------------------|----------------|-----------------------------------------|
| 10 | Sodium salt.....     | 0.25           | 1.25                                    |
|    | Silver salt.....     | 1.0            | 1.30                                    |

The antiplumming agents in accordance with our invention may also be employed in layers which are first laid down on the paper support such as baryta-gelatin 15 layers and the emulsion is applied thereover. Our invention is especially adapted for use in connection with photographic emulsions employed for photographic paper purposes in which drying at elevated temperatures occurs.

We claim:

- 20 1. A photographic element comprising a silver halide emulsion layer, containing as an additive thereto an antiplumming agent selected from the group consisting of the silver salt of thioglycolylamidobenzothiazole and the silver salt of acetylthioglycolylamidobenzothiazole.
- 25 2. A photographic element comprising a silver halide emulsion layer containing as an additive thereto a sufficient proportion therein of a compound selected from the group consisting of the silver salt of thioglycolylamidobenzothiazole and the silver salt of acetylthioglycolylamidobenzothiazole to prevent plumping of the photographic image formed therefrom.
- 30 3. A photographic element comprising a silver halide emulsion layer and in contact therewith a water permeable colloid layer containing as an additive thereto an antiplumming agent selected from the group consisting of the silver salts of thioglycolylamidobenzothiazole and the silver salts of acetylthioglycolylamidobenzothiazole.
- 35 4. A photographic silver halide emulsion containing as an additive thereto the silver salt of thioglycolylamido-40 benzothiazole in sufficient amount to prevent plumping of the photographic image which is formed by the emulsion.
- 45 5. A photographic silver halide emulsion containing as an additive thereto the silver salt of acetylthioglycolylamidobenzothiazole in sufficient amount to prevent plumping of the photographic image which is formed by the emulsion.
- 50 6. A coating composition comprising an aqueous solution of gelatin containing as an additive thereto a compound selected from the group consisting of the silver salts of thioglycolylamidobenzothiazole and of acetylthioglycolylamidobenzothiazole.

References Cited in the file of this patent

UNITED STATES PATENTS

- 2,214,446 Albers et al. Sept. 10, 1940  
 2,432,865 Dimsdale et al. Dec. 16, 1947  
 2,657,135 Lowe et al. Oct. 27, 1953

FOREIGN PATENTS

- 436,576 Great Britain Jan. 6, 1934  
 484,595 Great Britain May 9, 1938  
 699,858 Great Britain Nov. 18, 1953  
 708,065 Great Britain Apr. 28, 1954